

(No Model.)

J. H. GUEST.

FORMING AND TREATING ELECTRICAL CARBONS.

No. 256,213.

Patented Apr. 11, 1882.



Witnesses;

C. B. Perkins  
Geo. E. Marvin

Inventor;  
John H. Guest  
Attorney  
New York

# UNITED STATES PATENT OFFICE.

JOHN H. GUEST, OF BROOKLYN, NEW YORK.

## FORMING AND TREATING ELECTRICAL CARBONS.

SPECIFICATION forming part of Letters Patent No. 256,213, dated April 11, 1882.

Application filed September 7, 1881. (No model.)

*To all whom it may concern:*

Be it known that I, JOHN H. GUEST, of Brooklyn, Kings county, New York, have invented certain new and useful Improvements 5 in Forming and Treating Electrical Carbons, of which the following is a specification.

This invention relates more especially to the production of carbon loops for incandescent electric lamps; and it consists partly in a special form of such loop and in a mode of treating the loops so as to perfect the same and increase their hardness and permanency, and also to enlarge the attaching ends or "heels" of the loop for better attachment with the circuit-wires, as hereinafter fully set forth.

Carbon loops, as is well known, have been treated with an electro-deposit of carbon to harden and strengthen the same, which has been done both before and after the loop was 20 attached to its circuit-wires and inclosed in its enveloping exhausted globe, and the deposit of carbon has in some cases been uniform throughout the loop, while in other cases it has been increased or enlarged at the attaching 25 ends. In my system I employ these expedients, but in a somewhat different manner, whereby improved results are attained, as hereinafter set forth.

In the annexed drawings, Figure 1 represents my improved carbon loop just after the 30 same has been carbonized, and Fig. 2 shows the same after treatment to perfect the same and enlarge its ends by the electro-deposit of hard carbon. Fig. 3 represents the third stage 35 in the manufacture of the loop, with the circuit-wires applied thereto, and Fig. 4 represents the finished stage with the attachment of the circuit-wires completed. Fig. 5 presents a sectional elevation of an apparatus em- 40 ployed in treating the carbon loops.

I prefer to form the carbon loops in the shape shown in Fig. 1, as this is advantageous and constitutes one feature of my invention. This loop may be described as of oval or circular 45 form, bent in upon itself at the middle, forming a secondary or minor loop within the outer or larger one, the shape being hence that of two concentric arches joined at their bases. This shape, as may be observed, has the ad- 50 vantage of including a long filament in a compact space, and, moreover, is strong and sub-

stantial, for it will be observed that both parts of the loop tend to re-enforce or balance each other. Thus the tendency of the inner arch is to fall down and spread the outer arch, while 55 the latter tends itself to fall in or close together and to counteract the tendency of the inner arch, thus rendering the whole form strong and stable. This loop may be formed from any suitable carbonaceous material, fibrous or 60 otherwise; but I prefer to form it from a slender strip or filament of bamboo, which strip is at first reduced to the proper size and shape by draw-plates or other reducing-tools previous to carbonizing. The filament thus reduced is next bent into the described shape, 65 as shown in Fig. 1, and is placed between two closely-fitting iron plates, which are thence placed in a furnace or crucible and subjected to a high heat to thoroughly carbonize the filament, after which the plates are withdrawn 70 and cooled and the carbonized loop removed, when it will appear as shown in Fig. 1. One of the aforesaid iron plates is studded with a number of curved projections or circular pins 75 so disposed as to correspond to the form of the loop, so that the bamboo strip is easily curved into the proper shape by simply bending it around the projections previous to clamping the two plates together.

The bamboo filament from which the loop is made is necessarily of uniform size throughout, whereas it is desirable to have the ends of the finished loop where the circuit-wires attach thicker than the rest. It will be also understood that although the bamboo strip from which the loop is formed be of uniform thickness, yet after this strip has been carbonized it will frequently show many irregularities, being thin at some parts and thick at others, 90 whereas it is quite important that the part of the loop which is to become incandescent should be as uniform as possible throughout. To effect these results it has been usual to heat the carbonized filament to incandescence in an atmosphere containing some carbon compound, either by the passage of an electric current, or otherwise, which produces a deposit of carbon on the filament, and an increased deposit has been produced on the heels or ends of the 95 filaments to enlarge the same.

In Fig. 5 is shown a sectional elevation of

my apparatus for performing these operations, in which *a* represents a suitable base, from the center of which rises a form of Argand gas-burner, *b c*. This burner consists of an outer 5 tube or cylinder, *b*, into the bottom of which hydrocarbon gas may be admitted through the pipe and cock shown, and an inner cylinder or cup, *c*, which depends into the former and is closed at its bottom but open at the top. 10 Space is left between the two tubes, as shown, through which the gas may freely rise, and the top edges of the two tubes terminate nearly on a level and closely approach, so as to leave a narrow annular space between them to allow 15 the escape of a narrow annular jet of gas, similar to the jet of an Argand burner, with the difference, however, that no air is admitted into the middle of the flame. The inner cup is preferably corrugated on its sides, and is capable 20 of being easily lifted out of the tube *c*, and its mouth is preferably flared to rest on a few short projections in the mouth of the tube *b*, so as to be supported in central position in the gas-tube *b*, yet leave an annular jet-space 25 between the edges thereof, as will be understood.

From the base on each side of the gas-burner arise two tubular pillars, *d d'*, into which fit two adjustable standards, *e e'*, which are joined 30 in parallel rigid position by a cross-bar, *f*, which is curved at its middle to pass around the burner *b*, so that the standards are thus held firmly together and may be adjusted up or down as one part in the pillars *d d'*, and held 35 at any desired position by the clamp-screws *g g*. Now, from the top of the standards *e e'* tweezers or forceps *h h'* project toward each other, and the tips of their jaws approach each other over the gas-burner and over the mouth 40 of the cup *c*, as shown.

In preparing to treat a carbon loop the standards *e e'* and their attachments are raised or removed from the pillars *d d'*, and the ends of the freshly-carbonized loop as it appears in 45 Fig. 1 are clamped in the respective forceps *h h'*, and the standards, &c., are then adjusted in position, so that the loop hangs into the cup *c*, as shown in Fig. 5. Now, the pillars *d d'*, standards *e e'*, and the forceps *h h'* are of 50 course made of metal or some conducting material, and they are respectively insulated from each other, and the negative wire from a dynamo-machine or other source of electricity is connected with one of the pillars and the positive 55 wire with the other pillar, so that if the circuit be closed the loop will form part of the circuit, and may be raised to incandescence by the passage of the current. A circuit-closing device should be used which will admit of 60 turning the current on gradually, so as to raise the loop to any desired degree of incandescence, or to gradually increase its incandescence, as will be understood. Now, when the carbon loop is clamped and adjusted into the 65 position as already described and shown in Fig. 5, but before the circuit is closed on the

same, the gas is turned on in the burner *b* and ignited at the edge of the same, where it will form in a cone of flame above the cup *c*, as illustrated. The heat of the flame being rapidly 70 communicated to the burner *b* and cup *c*, the air in the latter will be rarefied, and will gradually diffuse with the gas from the interior of the flame, which gas will soon fill the cup *c* and displace the air, so as to form a hydrocarbon atmosphere around the carbon loop. In 75 most cases, however, I prefer to increase the richness of this atmosphere by a small quantity of liquid hydrocarbon, preferably kerosene, either dropped into the bottom of the cup *c* or 80 smeared by a brush on its sides, which liquid will soon vaporize and envelop the carbon loop with a rich carbonaceous atmosphere. When the atmosphere is thus formed around the loop, which will occur in a short time after 85 the gas is lighted, the circuit is closed on the loop gradually, or rather with gradually-increasing strength of current. It is to be here noted, however, that according to my system the current is not sent at first through 90 the entire loop, but in a short circuit only through the ends or heels *n n* by means of a platinum wire, *i*, which rests lightly as a conducting bridge from heel to heel, as shown in Fig. 5, which wire is attached to an adjustable arm, *m*, having both a vertical and swinging adjustment on the standard *e*, in the manner illustrated, and preferably insulated from the standard. Hence when the circuit is now closed the heels of the carbon loop 95 will be rendered incandescent, and the hydrocarbon atmosphere around them will become decomposed, and a deposit of fine hard carbon possessing a metallic quality and appearance will be formed on the heels, and this action is 100 allowed to continue till the heels become considerably enlarged and strengthened by a thick layer of the deposit, as seen in Fig. 5. When thus sufficiently enlarged the circuit is broken and the wire *i* removed from the loop. The 105 current is now turned on gradually, so as to pass through the entire loop, raising the slender parts or loop proper to incandescence. The thinner portions of the luminous loop will now be seen to possess a greater degree of incandescence than the thicker parts, and the deposit will form on the parts in proportion to their degree of incandescence, so that the thinner parts will become rapidly built up so as to 110 cure or neutralize its defects, and thus render 115 the loop of uniform size, and at the same time strengthen and harden it with a film of compact carbon having a metallic quality. When, therefore, the loop is seen to show a uniform luminous color throughout, as near as the eye 120 can judge, the treatment is complete, and the circuit may then be broken and the loop removed, when it will appear as shown in Fig. 2, after which other loops may be treated in the same manner and in a rapid and easy way 125 by this simple and efficient system. After the treatment of the loop is finished, as in Fig. 2,

it is next attached in any suitable manner, as shown in Figs. 3 and 4, to the circuit-wires, which may be either platinum or copper.

I prefer to make the circuit-wires where they attach to the loop of copper, and to connect these copper wires at a little distance from the loop with platinum wires; but, if desired, platinum wires alone may be used.

For the purpose of electric lamps a loop form of the carbon is of course preferable; but my system of treatment herein set forth is not of course confined to looped forms, but is equally adapted to straight or other forms of carbon filaments.

15 In lieu of the gas-burner shown for providing the carbon atmosphere, an oil-burner of similar form may be used; but it is not so desirable.

What I claim is—

20 1. An apparatus for treating electrical carbons, consisting of a burner adapted to emit a hollow flame, and means for holding a carbon within the hollow or the gases of the flame, and means for passing an electric current through 25 said carbon or rendering it incandescent in the gases of said flame, substantially as herein set forth.

2. An apparatus for treating electrical carbons, consisting of a burner of Argand or tubular form adapted to emit a hollow or tubular 30 flame, with a space or receptacle within the tubular burner freely open at the top to admit and inclose the carbon loop and permit observation of the same while under treatment, with electric-circuit connections and clamping devices external to said burner to hold the carbon within said receptacle and to include the same in an electric circuit, substantially as herein shown and described. 35

3. An apparatus for treating electrical carbons or carbon loops, consisting of a burner adapted to emit a hollow carbonaceous flame, in combination with adjustable forceps mutually insulated and adapted to respectively seize each end of the carbon and hold it in the hollow or gases of the flame, and means for including said forceps and the carbon held thereby in an electrical circuit, substantially as herein set forth. 40 45

JOHN H. GUEST.

Witnesses:

CHAS. M. HIGGINS,  
JNO. E. GAVIN.